

## UNITED STATES PATENT OFFICE

2,038,639

## METHOD OF PRODUCING CASTINGS

Charles O. Burgess, New York, N. Y., assignor, by  
mesne assignments, to Union Carbide and  
Carbon Corporation, a corporation of New  
York

No Drawing. Application July 26, 1933,  
Serial No. 682,275

4 Claims. (Cl. 75—127)

The invention relates to a method of producing castings which are characterized by improved strength, ductility and machinability.

It is well known that additions to cast iron of certain carbide forming elements, for example, those of the group consisting of chromium, tungsten, vanadium, and titanium, tend to impart increased hardness, strength, wear resistance, and heat resistance. However, the addition of these elements tends to harden cast iron, and to decrease materially its ductility and machinability; hence for many purposes the amount of the carbide forming elements that may be added is limited.

15 The present invention is based on the discovery that the hardening effect of carbide forming elements is decreased, and the strength, ductility, and machinability of the casting are improved, if a substantial amount of a graphitizing agent,

any given casting composition without decreasing or destroying machinability.

All cast irons containing more than about 1% carbon may be benefited by the use of the invention. In general, the final composition of the 5 casting should be substantially 1% to 4% carbon, 1% to 4% graphitizing agents, 0.15% to 1% manganese, up to about 0.5% sulfur, 0.05% to 0.3% phosphorus, 0.1% to 35% carbide forming elements, remainder iron. The greatest use of 10 the invention may be in producing castings containing 0.1% to 2% chromium as the carbide forming element; but the improvement in properties is found to be marked in castings containing up to 35% and more chromium or other 15 carbide forming element.

The table given below is illustrative of the improvement in the properties of cast iron attainable according to the invention:

| 20 | Casting number | Ladle addition       | Analysis of casting |      | Transverse tests |           | Tensile strength, pounds | Hardness Brinell number | 25 |
|----|----------------|----------------------|---------------------|------|------------------|-----------|--------------------------|-------------------------|----|
|    |                |                      | % Cr                | % Si | Strength pounds  | Defl. in. |                          |                         |    |
| 25 | 1.....         | None.....            | Nil                 | 2.52 | 3,050            | 0.003     | 31,400                   | 179                     | 30 |
|    | 2.....         | 1% Cr.....           | 1.01                | 2.39 | 3,700            | 0.090     | 41,950                   | 315                     |    |
|    | 3.....         | 1% Cr, 1.38% Si..... | 1.00                | 2.42 | 5,025            | 0.153     | 66,550                   | 260                     |    |
|    | 4.....         | None.....            | 14.04               | 2.52 | 3,900            | 0.07      | .....                    | .....                   |    |
| 30 | 5.....         | 1.5% Si.....         | 14.59               | 2.42 | 4,900            | 0.085     | .....                    | .....                   | 30 |

for example, silicon, nickel, aluminum, or zirconium, is added to the molten iron shortly before the melt is cast rather than during the initial 35 melting period. The graphitizing agent is preferably added in the ladle.

When a graphitizing element is added in the above described manner shortly before pouring, a marked increase in strength, ductility, and machinability results, as compared to a casting having the same composition but treated with the graphitizing agent at a time other than shortly before pouring. The treatment also results in a marked refinement of the structure of the casting, and serves to break up or to inhibit the formation of large crystallites of carbides, which doubtless contributes to the improved machinability and strength of the castings. The best results are obtained when the amount of silicon 45 and other graphitizing agents present during the melting period is relatively low so that a large proportion of the total final silicon may be added immediately before casting.

The invention thus affords a means of increasing 50 the content of carbide forming element in

In general, the invention provides castings having a transverse test strength greater than about 4500 pounds, as compared to 3000-4000 pounds in iron castings previously known.

The analyses of castings 1, 2, and 3, respectively, were substantially identical with the exception of the chromium content of casting number 1. Likewise, the analyses of castings 4 and 5 were substantially identical. The silicon in castings numbers 1, 2 and 4 was added in the furnace in the usual manner; while part of the silicon in castings numbers 3 and 5 was added in the ladle. Casting number 3 was materially stronger, more ductile, and more easily machinable than casting number 2, and stronger, harder, and more wear resistant than casting number 1. Similarly, casting number 5 was materially stronger and more easily machinable than casting number 4.

The graphitizing agent may be added as a metal or a ferroalloy. The carbide forming agent may be added in the furnace or in the ladle, as a metal, ferroalloy, or compound. If chromium and silicon are both to be added in the ladle, the addition may conveniently be made as a silicon-

35

40

45

50

55

chromium alloy, or as a ferrochromium-silicon alloy, or as a low melting copper, chromium, silicon alloy.

I claim:

- 5 1. Method of producing a ferrous alloy casting having substantially the composition: 0.1% to 35% chromium, 1% to 4% silicon, 1% to 4% carbon, 0.15% to 1% manganese, up to about 0.3% phosphorus, the remainder iron, and characterized by improved machinability, ductility, and strength, which comprises forming a melt the silicon content of which is materially less than is desired in the casting, adding silicon, and casting 10 the melt substantially immediately after the addition of silicon.
- 10 2. Method of producing a ferrous alloy casting having substantially the composition: 0.1% to 15% chromium, 1% to 4% silicon, 1% to 4% carbon, 0.15% to 1% manganese, up to about 0.5% sulfur, up to about 0.3% phosphorus, the remainder iron, and characterized by improved machinability, ductility, and strength, which comprises forming a melt the silicon content of which is materially less than is desired in the casting, adding silicon, and casting 15 the melt substantially immediately after the addition of silicon.
- 15 20 25

3. Method of producing a ferrous alloy casting having substantially the composition: 0.1% to 2% chromium, 1% to 4% silicon, 1% to 4% carbon, 0.15% to 1% manganese, up to about 0.5% sulfur, up to about 0.3% phosphorus, the remainder iron, 5 and characterized by improved machinability, ductility, and strength, which comprises forming a melt the silicon content of which is materially less than is desired in the casting, adding silicon, and casting the melt substantially immediately 10 after the addition of silicon.

4. Method of producing an alloyed cast-iron casting containing from 0.1% to 15% chromium which comprises forming a melt of chromium-alloyed iron the silicon content of which is materially less than is desired in the casting, adding silicon, and casting the melt substantially immediately after the addition of silicon, whereby is produced a casting having a structure consisting chiefly of a pearlitic ground mass, small graphite 20 flakes, and small widely dispersed non-dendritic carbide particles distributed substantially uniformly throughout the ground mass the proportion of carbide present being only a minor fraction of that normally present in cast iron of 25 similar composition.

CHARLES O. BURGESS.